# EUROPEAN PATENT SPECIFICATION

(11) **EP 0 222 507 B1**
(45) Date of publication and mention of the grant of the patent: **13.12.1989**
(21) Application number: 86307817.6
(22) Date of filing: 09.10.1986
(51) Int. Cl.: H01B 7/02, H01B 3/44

(54) **Shaped articles of crosslinked polymers**
Formteile aus vernetzten Polymeren
Pièces moulées de polymères réticulés

(30) Priority: 11.10.1985 US 786806
(43) Date of publication of application: 20.05.1987
(73) Proprietor: RAYCHEM CORPORATION (a Delaware corporation), Menlo Park, California 94025 (US)
(72) Inventor: Lunk, Hans E., Menlo Park California 94025 (US); Mehan, Ashok, Union City California 94587 (US); Enault, Neal, Sunnyvale California 94086 (US)
(74) Representative: Dlugosz, Anthony Charles

(56) References cited:
- CA-A- 1 151 255
- US-A- 3 852 518
- US-A- 4 155 823
- US-A- 4 310 597
- US-A- 4 353 961

## Description

This invention relates to insulated electrical conductors.

It is known to use cross-linked polymeric compositions as electrical insulation on a wire or other conductor. Known insulated wires include wires coated with a layer of a radiation cross-linked fluorocarbon polymer, particularly an ethylene/tetrafluoroethylene copolymer (often referred to as an ETFE polymer), which are extensively used for the wiring in aircraft. Military Specification No. MiL-W-22759 sets various standards for such standards for such insulated wires. Reference may be made for example to U.S. Patents Nos. 3 763 222,3 840 619,3 894118,3 911 192, 3 970 770, 985 716,3 995 091,4 031 167,4 155 823 and 4 353 961. Such wires have the significant disadvantage that if the outer surface of the insulation is damaged, subsequent flexing of the wire causes the damage to propagate through the insulation, at a rate which is highly undesirable. This disadvantage is especially serious when the insulated wire is to be used in an aircraft or in other high performance situations where the consequences of insulation failure can be so serious. A quantitative measure of this disadvantage can be obtained from a notch propagation test such as that described below.

We have discovered that this disadvantage can be substantially mitigated by insulation which comprises an inner layer of a polymer which has little cross-linking and an outer layer of polymer which has a relatively high level of cross-linking. Furthermore, this improvement is obtained with little or no substantial deterioration of other important properties of the insulation, for example, resistance to scrape abrasion, resistance to crossed wire abrasion and resistance to cut-through.

In one aspect, the present invention provides an insulated electrical conductor, especially a wire, which comprises:
(1) an electrical conductor; and
(2) electrical insulation which comprises:
   (a) an inner electrically insulating layer which (i) is composed of a first melt-processed, cross-linked polymer composition wherein the polymer comprises a fluorocarbon polymer having a melting point of at least 200_{°}C, and (ii) has a first M₁₀₀ value of 0 to 17.5 kg/cm² (0 to 250 psi); and
   (b) an outer electrically insulating layer which (i) is separated from the conductor by the inner layer, (ii) is composed of a second melt-processed cross-linked polymeric composition wherein the polymer comprises a fluorocarbon polymer having a melting point of at least 200_{°}C, and (iii) has a second Mice value which is at least 24.5 kg/cm2 (350 psi).

The M₁₀₀ values given herein are modulus values measured at a temperature above the melting point of the polymer by the procedure described in detail below, and therefore reflect the level of cross-linking in the layer.

A preferred method of making such an insulated conductor comprises:
(1) melt-extruding around the wire a first electrically insulating composition which comprises a fluorocarbon polymer having a melting point of at least 200_{°}C and 0-2% by weight of a radiation cross-linking agent, thereby forming a first insulating layer;
(2) melt-extruding around the first insulating layer a second electrically insulating composition which comprises a fluorocarbon polymer having a melting point of at least 200_{°}C and at least 5% by weight of a radiation cross-linking agent, thereby forming a second insulating layer;
(3) maintaining contact between the first and second layers under conditions such that part of the radiation cross-linking agent migrates from the second layer into the first layer; and
(4) without further addition of radiation cross-linking agent to the layers, irradiating the first and second layers to effect cross-linking thereof so that the first insulating layer has a first Mice value of less than 17.5 kg/cm² and the second insulating layer has a second M₁₀₀ value which is at least 24.5 kg/cm².

The polymeric component in the polymeric compositions used in the present invention preferably comprises, and more preferably consists essentially of, a melt-shapeable crystalline polymer having a melting point of at least 200_{°}C, preferably at least 250_{°}C, or a mixture of such polymers. The term "melting point" is used herein to denote the temperature above which no crystallinity exists in the polymer (or, when a mixture of crystalline polymers is used, in the major crystalline component of the mixture). The term "fluorocarbon polymer" is used herein to denote a polymer or mixture of polymers which contains more than 10%, preferably more than 25%, by weight of fluorine. Thus the fluorocarbon polymer may be a single fluorine-containing polymer, a mixture of two or more fluorine-containing polymers, or a mixture of one or more fluorine-containing polymers with one or more polymers which do not contain fluorine. Preferably the fluorocarbon polymer comprises at least 50%, particularly at least 75%, especially at least 85%, by weight of one or more thermoplastic crystalline polymers each containing at least 25% by weight of fluorine, a single such crystalline polymer being preferred. Such a fluorocarbon polymer may contain, for example, a fluorine-containing elastomer and/or a polyolefin, preferably a crystalline polyolefin, in addition to the crystalline fluorine-containing polymer or polymers. The fluorine-containing polymers are generally homo- or co-polymers of one or more fluorine-containing olefinically unsaturated monomers, or copolymers of one or more such monomers with one or more olefins. The fluorocarbon polymer has a melting point of at least 200_{°}C, and will often have a melting point of at least 250°C, e.g. up to 300°C. Preferably the polymeric composition has a viscosity of less than 105 poise at a temperature not more than 60_{°}C above its melting point. A preferred fluorocarbon polymer is a copolymer of ethylene and tetrafluoroethylene and optionally one or more other comonomers, especially a copolymer comprising 35 to 60 mole percent of ethylene, 35 to 60 mole percent of tetrafluoroethylene and up to 10 mole percent of one or more other comonomers. Other specific polymers which can be used include copolymers of ethylene and chlorotrifluoroethylene; copolymers of vinylidene fluoride with one or both of hexafluoropropylene and tetrafluoroethylene, or with hexafluoroisobutylene; and copolymers of tetrafluoroethylene and hexafluoropropylene.

The polymeric composition can optionally contain suitable additives such as pigments, antioxidants, thermal stabilisers, acid acceptors and processing aids.

The first and second compositions preferably contain the same polymeric components, and more preferably are substantially the same in all respects except for the level of cross-linking.

The conductor is preferably a metal (e.g. copper) wire, which may be stranded or solid. The wire may be for example from 10 to 26 AWG in size. The first layer preferably contacts the conductor. The second member is preferably also in the form of a layer which has the same general shape as the first layer or which serves to join together a number of wires each of which is surrounded by a first layer, thus forming a ribbon cable. The layers are preferably in direct contact, but may be joined together by a layer of adhesive.

The first and second members are preferably formed by melt-extrusion, particularly by sequential extrusion, which may be tubular or pressure extrusion, so that the layers are hot when first contacted, in order to promote migration of the cross-linking agent. The polymeric compositions should preferably be selected so that at least the outer layer has a tensile strength of at least 3,000 psi (210 kg/cm²); and since a higher tensile strength is usually desired in the cross-linked product and there is frequently a loss of tensile strength during the irradiation step, a higher initial tensile strength is preferred, e.g. greater than 6,000 psi (420 kg/cm²), preferably at least 7,000 psi (490 kg/cm2), particularly at least 8,000 psi (560 kg/cm2).

The thickness of the inner layer is generally 0.0075 to 0.038 cm (0.003 to 0.015 inch), preferably 0.0075 to 0.0225 cm (0.003 to 0.009 inch). The thickness of the outer layer is generally 0.01 to 0.063 cm (0.004 to 0.025 inch), preferably 0.01 to 0.023 cm (0.005 to 0.009 inch).

Preferred radiation cross-linking agents contain carbon-carbon unsaturated groups in a molar percentage greater than 15, especially greater than 20, particularly greater than 25. In many cases the cross-linking agent contains at least two ethylenic double bonds, which may be present, for example, in allyl, methallyl, propargyl or vinyl groups. We have obtained excellent results with cross-linking agents containing at least two allyl groups, especially three or four allyl groups. Particularly preferred cross- linking agents are triallyl cyanurate (TAC) and triallyl isocyanurate (TAIC); other specific cross-linking agents include triallyl trimellitate, triallyl trimesate, tetrallyl pyromellitate, the diallyl ester of 1,1,3-trimethyl-5-carboxy-3-(p-carboxyphenyl) indan. Other cross-linking agents which are known for incorporation into fluorocarbon polymers prior to shaping, for example those disclosed in U.S. Patents referenced above, can also be used. Mixtures of cross-linking agents can be used.

In the preferred method of preparing articles of the invention, in which cross-linking agent migrates from the second member to the first member, the first composition as extruded contains little or no cross- linking agent (e.g. 0 to 2% by weight, preferably 0%), and the second composition as extruded contains more than is desired during the cross-linking step, e.g. at least 5%, preferably 5 to 25%, particularly 7 to 12%, by weight. The time for which the layers should be maintained in contact prior to cross-linking depends upon the extent of migration which is needed and the temperature during such contact, which is preferably 5 to 150_{°}C below the melting point of the polymer (or the lower melting polymer if there are two or more polymers in the layers). At the time of irradiation, the inner layer preferably contains 0 to 3% by weight of cross- linking agent and the outer layer preferably contains 3 to 10% by weight of crosslinking agent.

The dosage employed in the irradiation step is generally below 50 Mrads to ensure that the polymer is not degraded by excessive irradiation, and the dosages preferably employed will of course depend upon the extent of cross-linking desired, balanced against the tendency of the polymer to be degraded by high doses of irradiation. Suitable dosages are generally in the range 2 to 40 Mrads, for example 2 to 30 Mrads, preferably 3 to 20 Mrads, especially 5 to 25 or 5 to 20 Mrads, particularly 5 to 15 Mrads. The ionising radiation can for example be in the form of accelerated electrons or gamma rays. Irradiation is generally carried out at about room temperature, but higher temperatures can also be used.

The inner layer preferably has an Mice value of at least 2.8 kg/cm2 (40 psi) and especially from 3.5 to 10.5 kg/cm² (50 to 150 psi). The elongation of the inner layer is preferably at least 100%, particularly at least 125%, e.g. at least 150%, especially 200 to 300%.

The outer layer is preferably cross-linked so that it has an Mice value of at least 28 kg/cm² (400 psi), particularly at least 31.5 kg/cm² (450 psi), with yet higher values of at least 42 kg/cm² (600 psi) being valuable in many cases. The elongation of the outer layer is preferably 40 to 150%, particularly 50 to 120%.

The various physical properties referred to in this specification are measured as set out below.

The Notch Propagation Values are measured on a piece of insulated wire about 30 cm (12 inch) long. A notch is made in the insulation, about 5 cm (2 inch) from one end, by means of a razor blade at right angles to the axis of the wire. The depth of the notch is controlled by mounting the razor blade between two metal blocks so that it protrudes by a distance which is 0.01 cm (0.004) inch or., if the insulation comprises two layers and the outer layer has a thickness t which is less than 0.018 cm (0.007 inch) thick, by a distance which is (t-0.0051) cm [(t-0.002) inch]. The end of the wire closer to the notch is secured to a horizontal mandrel whose diameter is three times the outer diameter of the insulation. A 0.675 kg (1.5 Ib) weight is secured to the other end of the wire so that the wire hangs vertically. The mandrel is then rotated clockwise, at about 60 revolutions a minute, until most of the wires has wrapped around the mandrel. The mandrel is then rotated, counterclockwise, until the wire has unwrapped and most of the wire has again been wrapped around the mandrel. The mandrel is then rotated clockwise until the wire has unwrapped and most of the wire has again been wrapped around the mandrel. This sequence is continued until visual observation of the notched area shows the conductor to be exposed. If, at this time, the conductor is broken (or some or all of the strands of a stranded wire conductor are broken) then the failure is attributable to that breakage, not to propagation of the notch through the insulation. The number of cy- des (half the number of times the rotation of the mandrel is reversed) is recorded.

The M₁₀₀ values are determined by a static modulus test as described in U.S. Patent No. 4,353,961 carried out at about 40°C above the melting point of the polymer, (e.g. at about 320_{°}C for ETFE polymers).

The tensile strengths and elongations are determined in accordance with ASTM D 638-72 (i.e. at 23_{°}C) at a testing speed of 50 mm (2 inch) per minute.

The cross-wire abrasion values, the cut-through resistance values, and the scrape abrasion values, are measured by the tests described in U.S. Patent No. 4,353,961.

The invention is illustrated by the following Examples, in which Example 1 is a comparative Example.

### Example 1

A 20 AWG (19/32) stranded tin-coated copper wire was insulated by melt-extruding over it, by sequential extrusion, an inner insulating layer 0.01 to 0.0125 cm (0.004 to 0.005 inch) thick and an outer insulating layer .018 to 0.020 cm (0.007 to 0.008 inch) thick. The layers were composed of the following compositions:

The polymeric insulation was cross-linked by irradiating it to a dosage of 14 Mrads.

### Example 2

The procedure of Example 1 was followed except that the composition of the inner layer was

The products of the Examples were subjected to the various tests described above and the following results (averaged for a number of specimens) were obtained.

## Claims

1. An insulated electrical conductor, especially a wire, which comprises:
(1) an electrical conductor; and
(2) electrical insulation which comprises:
(a) an inner electrically insulating layer which (i) is composed of a first melt-processed, cross-linked polymer composition wherein the polymer comprises a fluorocarbon polymer having a melting point of at least 200°C, and (ii) has a first M₁₀₀ value of 0 to 17.5 kg/cm² (0 to 250 psi); and
(b) an outer electrically insulating layer which (i) is separated from the conductor by the inner layer, (ii) is composed of a second melt-processed cross-linked polymeric composition wherein the polymer comprises a fluorocarbon polymer having a melting point of at least 200°C, and (iii) has a second Mioo value which is at least 24.5 kg/cm² (350 psi).

2. An insulated conductor according to claim 1, wherein the polymer in at least one of the first and second polymeric compositions consists essentially of a crystalline copolymer of 35 to 60 mole percent of units derived from ethylene, 35 to 60 mole percent of units derived from tetrafluoroethylene and 0 to 10 percent of units derived from at least one additional copolymerizable comonomer.

3. An insulated conductor according to claim 1 or 2, wherein the inner layer has an Mioo value of 2.8 to 17.5 kg/cm² (40 to 250 psi), preferably 3.5 to 10.5 kg/cm² (50 to 150 psi), and the outer layer has an M₁₀₀ value of at least 28 kg/cm² (400 psi), preferably at least 42 kg/cm² (600 psi).

4. An insulated conductor according to any one of the preceding claims wherein the inner layer has an elongation of at least 100%, preferably 200 to 300%, and the outer layer has an elongation of 40 to 150%, preferably 50 to 120%.

5. An insulated conductor according to any one of the preceding claims wherein the conductor is a metal wire; the inner layer contacts the wire, is 0.0075 to 0.038 cm (0.003 to 0.015 inch) thick and has an elongation of at least 125%; and the outer layer contacts the inner layer, is 0.01 to 0.063 cm (0.004 to 0.025 inch) thick and has an elongation of 50 to 120%.

6. An insulated conductor according to any one of the preceding claims wherein each layer has been cross-linked by irradiation with the aid of at least one of triallyl cyanurate and triallyl isocyanurate.

7. A process for the preparation of an insulated conductor as claimed in any one of the precedings claims which comprises:
(1) melt-extruding around a wire a first electrically insulating composition which comprises a fluorocarbon polymer having a melting point of at least 200_{°}C and 0.2% by weight of a radiation cross-linking agent, thereby forming a first insulating layer;
(2) melt-extruding around the first insulating layer a second electrically insulating composition which comprises a fluorocarbon polymer having a melting point of at least 200_{°}C and at least 5% by weight of a radiation cross-linking agent, thereby forming a second insulating layer;
(3) maintaining contact between the first and second layers under conditions such that part of the radiation cross-linking agent migrates from the second layer into the first layer; and
(4) without further addition of radiation cross-linking agent to the layers, irradiating the first and second layers to effect cross-linking thereof so that the first insulating layer has a first Mice value of less than 17.5 kg/cm² and the second insulating layer has a second M₁₀₀ value which is at least 24.5 kg/cm2.

8. A process according to claim 7, wherein the first polymeric composition is substantially free of radiation cross-linking agent when it is melt-shaped and the second polymer composition contains at least 5% by weight of radiation cross-linking agent immediately after it has been melt-shaped.

## Revendications

1. Conducteur électrique isolé, notamment un fil, comprenant:
(1) un conducteur électrique; et
(2) un isolant électrique comportant:
(a) une couche intérieure électriquement isolante, qui (i) est formée par une première composition polymérique réticulée traitée par fusion, dans laquelle le polymère est constitué par un polymère fluorocarboné possédant un point de fusion égal au moins à 200_{°}C, et (ii) possède une première valeur M₁₀₀ comprise entre 0 et 17,5 kg/cm² (0 à 250 psi); et
(b) une couche extérieure électriquement isolante, qui (i) est séparée du conducteur par la couche intérieure et (ii) est formée par une seconde composition polymérique réticulée traitée par fusion, dans laquelle le polymère est constitué par un polymère fluorocarboné possédant un point de fusion égal à au moins 200_{°}C, et (iii) possède une seconde valeur Mₗoo égale à au moins 24,5 kg/cm² (350 psi).

2. Conducteur isolé selon la revendication 1, dans lequel le polymère présent dans au moins l'une des première et seconde compositions polymériques est constitué essentiellement par un copolymère cristallin contenant 35 à 60 pour cent en moles d'unités dérivées de l'éthylène, 35 à 60 pour cent en moles d'unités dérivées du tétrafluoroéthylène et 0 à 10 pour cent d'unités dérivées d'au moins un comonomère co- polymérisable additionnel.

3. Conducteur isolé selon la revendication 1 ou 2, dans lequel la couche intérieure possède une valeur M₁₀₀ comprise entre 2,8 et 17,5 kg/cm² (40 à 250 psi), de préférence entre 3,5 et 10,5 kg/cm² (50 à 150 psi), et la couche extérieure possède une valeur M₁₀₀ égale à au moins 28 kg/cm² (400 psi), de préférence au moins 42 kg/cm2 (600 psi).

4. Conducteur isolé selon l'une quelconque des revendications précédentes, dans lequel la couche intérieure possède un allongement égal à au moins 100%, de préférence compris entre 200 et 300%, et la couche extérieure possède un allongement compris entre 40 et 150% et de préférence entre 50 et 120%.

5. Conducteur isolé selon l'une quelconque des revendications précédentes, dans lequel le conducteur est un fil métallique; la couche intérieure est en contact avec le fil et possède une épaisseur comprise entre 0,0075 et 0,038 cm (0,003 à 0,015) pouce), un allongement égal à au moins 125%; et la couche extérieure est en contact avec la couche intérieure et possède une épaisseur comprise entre 0,01 et 0,063 cm (0,004 et 0,025 pouce) et un allongement compris entre 50 et 120%.

6. Condcuteur isolé selon l'une quelconque des revendications précédentes, dans lequel chaque couche a été réticulée par irradiation à l'aide au moins du cyanurate de triallyle et de l'isocyanurate de triallyle.

7. Procédé pour préparer un conducteur isolé selon l'une quelconque des revendications précédentes, qui consiste à:
(1) appliquer au moyen d'une extrusion avec fusion, autour d'un fil, une première composition électriquement isolante qui comprend un polymère fluorocarboné possédant un point de fusion égal à au moins 200_{°}C et contient 0-2% en poids d'un agent de réticulation sous rayonnement, de manière à former un premier conducteur isolant;
(2) déposer au moyen d'une extrusion avec fusion, autour de la première couche isolante, une seconde composition électriquement isolante comprenant un polymère fluorocarboné possédant un point de fusion égal à au moins 200°C et au moins 5% en poids d'un agent de réticulation sous rayonnement, de manière à former une seconde couche isolante;
(3) maintenir le contact entre les première et les seconde couches dans des conditions telles qu'une partie de l'agent de réticulation sous rayonnement migre depuis la seconde couche dans la première couche, et
(4) sans aucune addition supplémentaire d'un agent de réticulation sensible au rayonnement aux couches, irradier les première et seconde couches de manière à obtenir leur réticulation de sorte que la première couche isolante possède une valeur Mᵢₒₒ inférieure à 17,5 kg/cm² et que la seconde couche isolante possède une seconde valeur Mₗₒₒ égale au moins à 24,5 kg/cm².

8. Procédé selon la revendication 7, dans lequel la première composition polymère est sensiblement exempte de l'agent de réticulation sous rayonnement, lorsqu'elle est moulée par fusion, et la seconde composition polymérique contient au moins 5% en poids de l'agent de réticulation sous rayonnement, aussitôt après qu'elle ait été moulée par fusion.

## Patentansprüche

1. Isolierter elektrischer Leiter, insbesondere Draht, der folgendes aufweist:
(1) einen elektrischen Leiter; und
(2) eine elektrische Isolierung, umfassend
(a) eine innere elektrisch isolierende Schicht, die
(i) aus einer ersten schmelzbearbeiteten, vernetzten polymeren Zusammensetzung besteht, wobei das Polymer ein Fluorcarbonpolymer mit einem Schmelzpunkt von mindestens 200_{°}C aufweist, und die
(ii) einen ersten Mioo-Wert von 0 bis 17,5 kg/cm² (0 bis 250 psi) hat; und
(b) eine äußere elektrisch isolierende Schicht, die
(i) durch eine innere Schicht vom Leiter getrennt ist,
(ii) aus einer zweiten schmelzbearbeiteten vernetzten polymeren Zusammensetzung besteht, wobei das Polymer ein Fluorcarbonpolymer mit einem Schmelzpunkt von mindestens 200_{°}C aufweist, und
(iii) einen zweiten Mioo-Wert von mindestens 24,5 kg/cm2 (350 psi) hat.

2. Isolierter Leiter nach Anspruch 1, wobei das Polymer in mindestens einer der ersten und zweiten polymeren Zusammensetzungen im wesentlichen aus einem kristallinen Polymer besteht, das 35 bis 60 Molprozent von Ethylen abgeleitete Einheiten, 35 bis 60 Molprozent von Tetrafluorethylen abgeleitete Einheiten, sowie 0 bis 10 Prozent Einheiten enthält, die von mindestens einem zusätzlichen copolymerisierbaren Comonomer abgeleitet sind.

3. Isolierter Leiter nach Anspruch 1 oder 2, wobei die innere Schicht einen Mloo-Wert von 2,8 bis 17,5 kg/cm² (40 bis 250 psi), vorzugsweise 3,5 bis 10,5 kg/cm² (50 bis 150 psi), und die äußere Schicht einen Mloo-Wert von mindestens 28 kg/cm² (400 psi), vorzugsweise mindestens 42 kg/cm2 (600 psi) aufweist.

4. Isolierter Leiter nach einem der vorangehenden Ansprüche, wobei die innere Schicht eine Dehnung von mindestens 100%, vorzugsweise 200 bis 300%, und die äußere Schicht eine Dehnung von 40 bis 150%, vorzugsweise 50 bis 120% aufweisen.

5. Isolierter Leiter nach einem der vorangehenden Ansprüche, wobei der Leiter ein Metalldraht ist und wobei die innere Schicht mit dem Draht in Kontakt steht, 0,0075 bis 0,038 cm (0,003 bis 0,015 Inch) dick ist und eine Dehnung von mindestens 125% aufweist; und wobei die äußere Schicht mit der inneren Schicht in Kontakt steht, 0,01 bis 0,063 cm (0,004 bis 0,025 Inch) dick ist und eine Dehnung von 50 bis 120% aufweist.

6. Isolierter Leiter nach einem der vorangehenden Ansprüche, wobei jede Schicht mit Hilfe von mindestens einer der Verbindungen Triallylcynanurat und Triallylisocyanurat durch Bestrahlung vernetzt worden ist.

7. Verfahren zur Herstellung eines isolierten Leiters nach einem der vorangehenden Ansprüche, das folgende Schritte umfaßt:
(1) Bildung einer ersten isolierenden Schicht durch Schmelzextrudieren einer ersten elektrisch isolierenden Zusammensetzung um einen Draht herum, wobei die erste elektrisch isolierende Zusammensetzung ein Fluorcarbonpolymer mit einem Schmelzpunkt von mindestens 200_{°}C ist und 0 bis 2 Gew.-% eines durch Strahlung vernetzenden Agens enthält;
(2) Bildung einer zweiten isolierenden Schicht durch Schmelzextrudieren einer zweiten elektrisch isolierenden Zusammensetzung um die erste isolierende Schicht herum, wobei die zweite isolierende Zusammensetzung ein Fluorcarbonpolymer mit einem Schmelzpunkt von mindestens 200_{°}C ist und mindestens 5 Gew.-% eines durch Strahlung vernetzenden Agens enthält;
(3) Aufrechterhalten des Kontaktes zwischen der ersten und der zweiten Schicht unter solchen Bedingungen, daß ein Teil des durch Strahlung vernetzenden Agens aus der zweiten Schicht in die erste Schicht hineinwandert; und
(4) Bestrahlung der ersten und der zweiten Schicht zur Durchführung der Vernetzung ohne weitere Zugabe von durch Strahlung vernetzendem Agens zu den Schichten, derart, daß die erste isolierende Schicht einen ersten Mioo-Wert von weniger als 17,5 kg/cm² und die isolierende Schicht einen zweiten Mioo-Wert von mindestens 24,5 kg/cm² erhält.

8. Verfahren nach Anspruch 7, wobei die erste polymere Zusammensetzung, wenn sie schmelzgeformt ist, im wesentlichen frei ist von durch Strahlung vernetzendem Agens, und die zweite polymere Zusammensetzung, unmittelbar nach dem sie schmelzgeformt wurde, mindestens 5 Gew.-% an durch Strahlung vernetzendem Agens enthält.
